

June 7, 1938.

C. B. WHITE

2,119,936

METHOD OF RECOVERING PURE COPPER FROM SCRAP AND RESIDUES

Filed Oct. 2, 1935



Inventor

C. B. White

Eugene C. Brown  
Attorney

## UNITED STATES PATENT OFFICE

2,119,936

METHOD OF RECOVERING PURE COPPER  
FROM SCRAP AND RESIDUES

Clarence B. White, Philadelphia, Pa.

Application October 2, 1935, Serial No. 43,277

1 Claim. (Cl. 204—57)

This invention relates to the recovery of electrolytically pure copper from scrap material, metallurgical by-products and residues containing metals in the form of alloys.

5 The primary object of the present invention is to eliminate the partial furnace refining which is employed at the present time in all metal recovery methods thereby simplifying the recovery of the copper content of commercial scrap alloy 10 materials and greatly reducing the expense.

The scrap materials and residues are first reduced in a blast or smelting furnace to separate the metals from the non-metallic contents. The molten metal is then cast directly into the form 15 of anode plates suitable for deposition in the electrolytic tanks. These cast anode plates may contain besides copper, various other metals, such as tin, lead, zinc, iron, antimony, nickel, bismuth, cadmium, gold, silver, platinum, etc.

20 The cast anodes are placed in the electrolytic tank in alternate arrangement with lead plates or other suitable nonsoluble cathodes, the anodes and cathodes being connected to a suitable source of current. When the copper of the anodes has 25 been deposited upon the lead cathodes, they are replaced by thin sheets of electrolytic copper and the current is then reversed to thereby transfer the copper previously plated upon the lead sheets to said thin copper sheets. The resulting 30 copper plate will be perfectly pure electrolytic copper, running over 99.97% pure.

My process of producing pure copper plates from commercial scrap material, metallurgical bi-products and residues will be more clearly 35 understood from the following description in connection with the accompanying drawing, in which—

Figures 1, 3, 4 and 5 are diagrammatic views illustrating the manner of obtaining electrolytically pure copper from cast metal plates obtained 40 from the smelting of the scrap metal; and Fig. 2 is a cross-sectional view on the line 2—2 of Fig. 1 showing the manner of suspending the plates in the tank.

45 In the first stage of my process the cast anodes A from the smelting furnace are suspended in the copper sulphate electrolyte in alternation with lead plates L, as shown in Fig. 1, the cast anodes being connected to the positive pole and the lead plates to the negative pole of the electrical source. The copper content of the anodes is deposited upon the lead plates, as outlined in broken lines, the anodes wasting away to a thin strip. Some of the metals, such as zinc and 50 iron, pass into solution while others form sul-

phates or other metallic salts and sink to the bottom of the tank as a sludge or slime.

The deficiency of copper in the electrolyte, (due to the fact that other metals than copper are removed from the cast anodes) is replenished periodically by adding copper sulphate or by passing the electrolyte over copper oxide as it is circulated by the usual circulating pump.

When substantially all of the copper has been deposited upon the lead plates and the cast 10 anodes have been reduced to a mere shell, the electrolyte is removed and the sludge is washed from the bottom of the tank. The lugs of the anodes with their attached cores may be returned to the scrap to be remelted. The metals 15 in solution and in the sludge or slimes may be recovered and the electrolyte purified as is well understood by metallurgists.

In the next stage of my process thin electrolytic copper sheets C<sup>2</sup> are substituted for the 20 cast anodes of the first stage and the tank is filled with fresh copper sulphate electrolyte as indicated in Fig. 3. The switch S is then reversed to cause the copper C<sup>1</sup> which was plated upon the lead plates during the first stage, to 25 now be transferred to the copper starting sheets C<sup>2</sup>. When substantially all of the copper has been removed from the lead plates and deposited upon the copper sheets C<sup>2</sup> as indicated in broken lines in Fig. 3, the resulting plates Cu, thus 30 formed are practically pure copper, running over 99.97% and having an electrical conductivity in excess of that required by commercial standards.

The thin copper sheet electrodes C<sup>2</sup> for starting the second stage or step in my process, may 35 be obtained by suspending a number of the cast anodes A, A<sup>1</sup> in the electrolytic tank and connecting them alternately to the opposite poles of the battery or electrical source, as indicated in Fig. 4, or preferably alternating the cast 40 anodes and lead plates as indicated in Fig. 5. When a thin copper sheet has been plated, the cathodes are removed and the plated sheets are stripped off to be used as the starting cathodes 45 in the second stage.

Instead of connecting the alternate plates forming the anodes and cathodes in multiple to the current source, it will be evident that they may be connected in a series circuit.

The advantages of my method of producing 50 plates of pure copper direct from smelted scrap metal will be appreciated from the above description of my process. The plates cast from the molten scrap metal of the smelting furnace are introduced immediately into the electrolytic 55

tank as anodes from which the pure copper is electrolytically extracted and plated upon lead or other insoluble electrodes and from the latter by reversing the current, said plated copper is 5 deposited upon thin sheets of electrolytic copper.

10 I have eliminated the steps of furnace refining heretofore employed and produce plates composed of electrolytically pure copper throughout.

I claim:

10 The method of producing pure copper from copper bearing scrap and metallurgical residues, which comprises smelting said scrap and residues to separate the metals from the non-metal content, casting the molten metal into plates to form 15 anodes, arranging said anodes in alternate rela-

tion with insoluble cathodes in a copper sulfate electrolyte, connecting the anodes and cathodes to the positive and negative poles respectively of a source of electric current until substantially all the copper content of the anodes is deposited 5 upon the cathodes the cast anodes being reduced to a thin strip or shell, removing the electrolyte and sludge, replacing the strip or shell with a sheet of electrolytic copper, adding fresh copper sulfate electrolyte and reversing the polarity of 10 the current from said source to the electrodes to thereby transfer the copper deposited upon the cathodes to said sheets to form plates of pure electrolytic copper.

CLARENCE B. WHITE. 15